

May 23, 1944.

H. C. MARTIN ET AL

2,349,365

FLEXIBLE ABRASIVE ARTICLE

Original Filed July 9, 1936



Fig. 1.



Fig. 2.



Fig. 3.



Fig. 4.



Fig. 5.



Fig. 6.



Fig. 7.

Fig. 8.



Fig. 9.

BY

INVENTORS.  
HARRY C. MARTIN.  
JOSEPH B. AUST.

*R. B. Martin*

ATTORNEY.

## UNITED STATES PATENT OFFICE

2,349,365

## FLEXIBLE ABRASIVE ARTICLE

Harry C. Martin and Joseph B. Aust, Niagara Falls, N. Y., assignors, by mesne assignments, to The Carborundum Company, Niagara Falls, N. Y., a corporation of Delaware

Application July 9, 1936, Serial No. 89,800  
Renewed September 26, 1938

12 Claims. (Cl. 51—197)

This invention relates to improved abrasive articles and a method of manufacturing the same. More specifically, the invention is concerned with flexible abrasive articles which are used in machines, such as abrasive belts and abrasive discs consisting of a flexible backing carrying a thin coating of abrasive grains attached to a surface thereof.

Although our invention is adapted to a number of embodiments, it is particularly addressed to the production of abrasive discs for use in surfacing metals such as the panels of automobile bodies and the like by the method described and claimed in a patent to Herbert R. Stratford No. 1,553,714. A second modification of the invention is concerned with abrasive belts or bands which are adapted to be mounted on pulleys or on wheels or drums.

We have illustrated our invention by a number of drawings wherein:

Fig. 1 is a partial section of a form of apparatus which we have employed in the use of our improved discs and illustrates the position of the disc when it is used;

Fig. 2 is a side elevation of a machine provided with a belt made in accordance with our invention;

Fig. 3 is a section of one form of our improved discs;

Fig. 4 is a section of the backing employed in the production of the disc illustrated in Fig. 1;

Figs. 5, 6, 7, 8 and 9 depict other structures of backings used in our invention.

Referring to Fig. 1, a disc 1, which forms part of the subject matter of the invention, is frictionally attached to a rotatable shaft 3 by the pressure applied to the disc by screwing the cap 5 into the shaft 3 so that the disc is squeezed against the backing element 7. The outer or working portion of the disc is yieldably supported by a pad 9 which is suitably attached to the backing element 7 and thereby to the shaft 3 to which the element 7 is fastened.

In use, the shaft 3 is rotated by means not shown in the drawing and the abrasive coated disc 1 is pressed against the outer surface of the disc 1 which is to be surfaced. In order to use such discs efficiently it is necessary to apply them to the work piece with considerable force and consequently the disc with its supporting pad 9 is subjected to rather severe stresses, both by reason of the pressure that is applied by the operator and by the torque that is transmitted through the shaft 3 and is occasioned by the drag of the abrasive grains on the work piece.

Heretofore, discs for use in this type of work have commonly been made using glue as the adhesive for attaching the grains to a backing of vulcanized fiber or hydrolyzed cellulose as described and claimed in a patent to Herbert R. Stratford No. 1,684,748. Such discs have been very successful and literally millions have been made and used. Their average abrading life on a standard test is about 9 minutes during which time they will remove an average of about 140 grams of steel.

Recent developments in the use of binders other than glue, such as heat hardenable synthetic resins, have made it possible to produce discs of this character which have a much longer abrading life and remove two to three times as much metal as the glue discs but such discs have been used only to a small extent because it has been necessary to employ spring steel for the backing and the cost of the articles has been correspondingly high.

When abrasive discs are made with a resin bond on the vulcanized fiber backings that have heretofore been used, difficulties are encountered 25 the nature of which depends upon the type of resin that is used and the details of the method employed to make the article. For example, the vulcanized fiber is weakened and made brittle by the temperatures that are required to satisfactorily cure some of the types of resin that have been found to be suitable as a binder or adhesive for the abrasive grains. Fiber is also hygroscopic and correspondingly susceptible to changes in atmosphere conditions and shrinks or expands with changes in the humidity of the atmosphere. When it is dried out it becomes brittle and if it is moistened it curls.

In Fig. 2 we have shown a form of machine which is commonly employed in using endless abrasive belts. The machine comprises a driven pulley 2, which is caused to rotate by a source of power not shown in the drawing, and a second pulley 4 about which is mounted a belt 6. The pulleys are mounted on shafts carried in suitable bearings supported by standards 8 and 10 respectively. A table 12 is usually provided to form a support for the belt at the part where the work is applied to the belt.

Belts for use on apparatus of this general type have commonly been made heretofore on a backing of paper or cloth. While such backings have been satisfactory where the grains have been bonded to the backings with glue, they are not well adapted for use with the improved binders discussed in the foregoing paragraphs. Either paper

or cloth is embrittled and weakened by prolonged heating at the temperatures employed to cure heat-hardenable resins, presumably because of a drying out of the fibers of the fabrics and possibly also because of some oxidation. Likewise, as was mentioned in discussing discs, the longer life of abrasives bonded with resins requires that the backings employed therewith shall be capable of withstanding the additional stresses caused by the prolonged use of the articles. It has therefore been found that the life of abrasive belts bonded with resins is often ended by failure of the backing before the coatings are worn out. Similar difficulties are experienced with abrasive bands which are mounted on drums as by stretching a band about the periphery of a drum and fastening the ends of the band in suitable clamps provided on the drum.

It is accordingly an object of the invention to provide an abrasive article and a backing therefor which shall not have the limitations of articles made heretofore as discussed above. Another object of the invention is to provide a method of making our improved abrasive articles. Another object of the invention is to provide an improved backing for flexible abrasive articles such as abrasive belts, bands and discs which shall be capable of withstanding the stresses and loads which are applied to such articles when they are used for long periods of time.

We have found that discs and bands made on a backing containing a sheet of plastic material reinforced with a suitable filler, preferably in the form of a sheet of cloth or paper, are eminently satisfactory for use for the purposes described. By selecting a suitable type of plastic such as a heat-hardened phenolic or alkyd resin, the backing will withstand the temperatures required to cure heat hardenable resins which have been found to be good adhesives for the abrasive grain. Other types of plastics, such as certain cellulose esters, have the required life when used but are not so well adapted for use with certain resins because of their tendency to soften under the temperatures used in curing the resin binder.

Compositions of the character just described are commonly called "plastics," even if they have been heat treated to harden them so that they are no longer fusible or soluble. Consequently, in claiming our invention, we have used this word "plastics" to indicate not only materials which may be soluble and fusible, and hence might be correctly called "plastics," but also heat-hardened products such as cured phenolic condensation products which were originally plastic but which would no longer be plasticizable either by heat or by the use of a solvent.

As illustrated in the drawing, our invention is adapted to a number of modifications, explanation of which will now be made.

In Fig. 3 we have shown a section of a completed disc made in accordance with one modification of the invention. In this drawing the plastic material 15 contains a layer of cloth 17 which is entirely embedded in the plastic. Attached to the upper surface of the plastic 15 is a second layer of cloth 19 (see also Fig. 4) to the outer surface of which abrasive grains 21 are attached by an adhesive 23.

Alternative backing structures shown in the drawing comprise:

Fig. 5—two layers of cloth 17 embedded in a plastic 15.

Fig. 6—a layer of wire cloth 25 embedded in a

sheet of plastic 15 and a layer of cloth 19 attached to a surface of the plastic.

Fig. 7—two sheets of paper 27 embedded in a sheet of plastic 15 and a surface layer of cloth 19 attached to the plastic 15.

Fig. 8—a sheet of plastic 15 containing a reinforcement of unwoven fibers 29 and having a sheet of cloth 19 attached to one of its surfaces.

Fig. 9—a sheet of cloth 17 and a sheet of paper 27 embedded in a sheet of plastic 15 and a layer of cloth 19 attached to a surface of the plastic 15.

One method which we have found to be suitable for preparing our improved backing material consists in first impregnating a sheet of reinforcing material, such as the cloth 17 of Figs. 3, 4 and 5 or the paper 27 of Fig. 7, with the plastic material 15, associating the impregnated sheet with a sheet of cloth 19 as shown in Figs. 4, 6, 7 and 8 or with a second impregnated sheet as shown in Fig. 5, and then subjecting the assemblage to heat and pressure to cause the plastic to flow into a continuous sheet 15 thereby enclosing the sheets 17 or 27 in the sheet 15 and also attaching the sheet 19 (where such is employed) to a surface of sheet 15.

This heat and pressure may be conveniently applied by placing the assemblage between the platens of a hot press of the character commonly used in making molded articles, or it may be passed around and between suitably heated rolls to cause the formation of the sheet 15.

The embedded sheets 17 or 27 may be impregnated with a plastic in any convenient manner as, for example, by dissolving the plastic in a suitable solvent, passing a web of the sheet through the solution of the plastic, and then evaporating the solvent. Where some forms of plastic which are obtainable in a normally liquid condition or which can be liquified by heating are employed, the use of a solvent may be dispensed with. Another method for forming the sheet of plastic material which is well adapted for use with the modification shown in Fig. 6, consists in casting the sheet 15 about the embedded sheet of reinforcement 25, the attached sheet 19 being associated with the sheet 15 either when the sheet 15 is cast or later, as for example, by moistening the surface of the plastic 15 with a suitable solvent to cause it to become adhesive and then associating the sheet of cloth 19, which may be previously sized with plastic if desired, with this adhesive surface.

In the embodiment of the invention which is illustrated in Fig. 8, a backing comprising the sheet of plastic material 15 containing a miscellany of fibers 29 and a surface coating of cloth 19 may be formed by first preparing a dry mixture of plastic material and fiber, distributing this in a suitable mold, spreading thereon a sheet of cloth 19 which has been preferably coated very lightly with a solution of the plastic 15 in a solvent, and then applying heat and pressure to fuse the plastic material 15 and cause it to form a continuous sheet and at the same time to adhesively attach the cloth 19 to the surface of the sheet of plastic material 15.

The backing material of our invention may be coated with abrasive grains by any convenient method. One method which we have found to be satisfactory, particularly where a disc is to be made with a coating of abrasive grains in the form of a band at and near the periphery as is frequently done, comprises first coating a surface of the backing at and near the periphery with an adhesive in liquid condition and then

applying to the adhesive coated surface a layer of abrasive grains which have been previously coated with an adhesive in a solid condition. For example, we may coat the backing with a normally liquid phenolic condensation product which is hardenable by heat to form a strong, tough bond, separately coat abrasive grains with a layer of heat-hardenable phenolic condensation product resin in the solid "A" stage, apply a thin layer of the resin coated grains to the resin coated surface of the backing, and then subject the article to heat treatment to harden the liquid resin and to cause the resin coatings on the grain to weld and unite with the resinous coating on the backing. The heat treatment required will depend upon the composition of the resinous materials employed. With commercial grades of phenol formaldehyde condensation products which we have used and which are commonly employed in the manufacture of abrasive articles, the coated article may be heated for about 12 hours gradually up to 300° F., followed by further heating for 6 hours at 300° F.

Another method which we have successfully employed in attaching the abrasive grains to the backing comprises the usual conventional method of making sandpaper. According to this method, the backing is first coated with a liquid adhesive material, a layer of abrasive grain is applied while the adhesive is still fluid enough to permit penetration by the grain, and an additional coating of adhesive is subsequently applied to secure the grains more firmly to the backing. In some cases it is customary to subject the article to a treatment to harden up the first or making coating of adhesive after the abrasive grains have been applied and before the second or sizing coating of adhesive is put on. The final operation is customarily a treatment to harden up the adhesive or binder coats.

As we have indicated above, the plastic material 15 may be of any suitable composition which will flow out into a continuous sheet which, when subjected to the stresses incident to the use of discs or bands, as previously described, will possess the required degree of flexibility and will not crack or be otherwise deficient in meeting the requirements of the service during the life of the abrasive article as determined by the effectiveness of the abrasive grains in removing material. We have found that phenolic condensation products, including oil-modified resins as well as the usual phenol-aldehyde resins, are quite satisfactory for our purpose. 55 We may also use other suitable materials such as certain alkyd resins, vinyl resins, or suitably plasticized cellulose esters or ethers such as cellulose acetate or ethyl cellulose, the selection of the plastic material being determined, to some extent, by the use to which the abrasive article is to be put. For example, an abrasive disc usually requires a less flexible backing than an abrasive belt.

Our invention is also adapted to the use of numerous adhesives for attaching the abrasive grains to the backing. One such adhesive which we have found to be quite suitable is the phenolic condensation product which we have described above. Other suitable binders are certain forms of alkyd resins, polyvinyl compounds such as polyvinyl alcohol and modified polyvinyl acetate wherein part of the acetate group has been replaced with an aldehyde such as acetaldehyde. Suitably plasticized cellulose esters 75

such as a cellulose nitrate lacquer containing cellulose nitrate and resin along with suitable plasticizing agents may also be employed as a binder for the abrasive grains.

5 Other modifications and embodiments of our invention will occur to those skilled in the art and may be practiced without departing from the spirit of the invention, the scope of which is defined by the appended claims.

10 We claim:

1. A flexible abrasive disc comprising a backing consisting of a sheet of heat-hardened phenolic resin containing a non-metallic reinforcement embedded within it and a layer of cloth firmly attached to a surface of the resin sheet, and a substantially single layer of abrasive grains bonded to the cloth by a heat-hardened phenolic resin, said disc being characterized by sufficient strength and stiffness so that it is adapted to 15 be driven from the center alone while being resiliently supported and by sufficient flexibility so that it can be bent while being applied to a workpiece in such a way that only a portion of the disc is in contact with the work at any given time and the remainder of the disc is disposed at an angle with respect to the working portion.

20 2. A flexible abrasive article comprising a backing consisting of a sheet of phenolic resin containing a non-metallic reinforcement embedded within it and a sheet of cloth attached to a surface of the sheet of resin, and a substantially single layer of abrasive grains attached to the sheet of cloth by a hardened resin bond, said bond extending through said cloth and uniting with the sheet of resin so as to form an article characterized by sufficient strength and stiffness so that a disc cut therefrom can be driven from the center alone while being resiliently supported and by sufficient flexibility so that it can be bent while being applied to a workpiece in such a way that only a portion of the disc is in contact with the work at any given time and the remainder of the disc is disposed at an angle with respect to the working portion.

25 3. A flexible endless abrasive band adapted for use in a surfacing machine and comprising a backing consisting of a sheet of plastic material containing a non-metallic reinforcement embedded within it and a sheet of cloth attached to a surface of the sheet of plastic material, and a substantially single layer of abrasive grains attached to the sheet of cloth by a hardened plastic bond, said bond extending through said cloth and uniting with the sheet of plastic material so as to form an article characterized by unusual strength of the backing and firm attachment of the abrasive grains to the backing.

30 4. A flexible abrasive disc comprising a backing consisting essentially of a sheet of heat-hardened phenolic resin containing a non-metallic cloth reinforcement embedded within it and a layer of cloth attached to a surface of the resin sheet, a substantially single layer of abrasive grains, and a heat-hardened phenolic resin attaching the abrasive grains to the layer of cloth and extending through the layer of cloth so as to form a substantially continuous body of heat-hardened phenolic resin extending from the back surface to the abrasive grains, said disc being characterized by sufficient strength and stiffness so that it can be driven from the center alone while being resiliently supported and by sufficient flexibility so that it can be bent while being applied to a workpiece in such a way that only a

portion of the disc is in contact with the work at any given time and the remainder of the disc is disposed at an angle with respect to the working portion.

5. The method of making flexible abrasive articles of the nature of sandpaper which comprises impregnating a sheet of non-metallic fabric with a liquid resinous material, applying a sheet of unimpregnated non-metallic fabric to one side of said impregnated sheet of fabric and adhesively uniting it therewith to form a laminated backing having one face formed by the impregnated fabric and the other face by the unimpregnated fabric, and thereafter applying a liquid resinous material to the unimpregnated fabric face, applying a layer of abrasive grain substantially one grain thick to such resinous coating, and heat-hardening the liquid resinous material.

6. A backing for abrasive discs comprising a disc of resin reinforced with fibers extending in random directions, said disc being cured from a single felted mass of resin impregnated fibers to resilient flexible condition by the application of heat and pressure, said disc having an integrally formed resin seal on all sides of said fibers and at the edges of said disc.

7. A flexible abrasive article comprising a backing consisting essentially of a sheet of plastic material containing a non-metallic reinforcement embedded within it and a sheet of cloth attached to a surface of the sheet of plastic material, and a substantially single layer of abrasive grains attached to the sheet of cloth by a hardened plastic bond, said article being characterized by sufficient strength and stiffness so that a disc cut therefrom can be driven from the center alone while being resiliently supported and by sufficient flexibility so that it can be bent while being applied to a workpiece in such a way that only a portion of the disc is in contact with the work at any given time and the remainder of the disc is disposed at an angle with respect to the working portion.

8. A flexible abrasive article comprising a backing consisting of a sheet of plastic material containing a non-metallic reinforcement embedded within it and a sheet of cloth attached to a surface of the sheet of plastic material, and a substantially single layer of abrasive grains attached to the sheet of cloth by a hardened plastic bond, said bond extending through said cloth and unit-

ing with the sheet of plastic material so as to form an article characterized by unusual strength of the backing and firm attachment of the abrasive grains to the backing.

9. A method of making flexible abrasive articles of the nature of sandpaper which comprises impregnating a sheet of non-metallic fabric with a liquid plastic material, applying a sheet of unimpregnated non-metallic fabric to one side of said impregnated fabric and adhesively uniting it therewith to form a laminated backing having one face formed by the impregnated fabric and the other face by the unimpregnated fabric, and thereafter applying a liquid plastic material to the unimpregnated fabric face, applying a layer of abrasive grain substantially one grain thick to such plastic coating, and hardening the liquid plastic material.

10. A method of making flexible abrasive products in the nature of sandpaper which comprises impregnating a sheet of non-metallic fabric with a liquid heat-hardenable phenolic resinous material, applying a sheet of unimpregnated non-metallic fabric to one side of said impregnated sheet of fabric and adhesively uniting it therewith to form a laminated backing having one face formed by the impregnated fabric and the other face by the unimpregnated fabric, and thereafter applying a liquid heat-hardenable phenolic resinous material to the unimpregnated fabric face, applying a layer of abrasive grains substantially one grain thick to such resinous coating, and heat-hardening the liquid resinous material.

11. An abrasive article comprising a backing having a layer of abrasive grains attached thereto by a resin bond, said backing comprising a sheet of resin reinforced with fibers extending in random directions, said sheet being cured from a mass of resin-impregnated fibers to resilient flexible condition by the application of heat and pressure.

12. An abrasive article comprising a backing having a layer of abrasive grains attached thereto by a hardened plastic bond, said backing comprising a sheet of plastic material reinforced with fibers extending in random directions, said sheet being cured from a mass of plastic-impregnated fibers to resilient flexible condition by the application of heat and pressure.

HARRY C. MARTIN.  
JOSEPH B. AUST.